# EUROPEAN PATENT SPECIFICATION

(11) **EP 1 888 803 B1**
(45) Date of publication and mention of the grant of the patent: **17.12.2014**
(21) Application number: 06733241.1
(22) Date of filing: 15.03.2006
(51) Int. Cl.: H05H 1/42, H05H 1/34, C23C 16/513

(54) **APPARATUS FOR GAS-DYNAMIC APPLYING COATINGS AND METHOD OF COATING**
VERFAHREN ZUM GASDYNAMISCHEN AUFBRINGEN VON BESCHICHTUNGEN UND BESCHICHTUNGSVERFAHREN
APPAREIL POUR L'APPLICATION GAZ DYNAMIQUE DE REVETEMENTS ET PROCEDE DE REVETEMENT

(30) Priority: 20.05.2005 RU 2005115327
(43) Date of publication of application: 20.02.2008
(73) Proprietor: OBSCHESTVO S OGRANICHENNOI OTVETSTVENOSTIJU OBNINSKY TSENTR POROSHKOVOGO NAPYLENIYA, Kaluzhskaya oblast, Obninsk 249031 (RU)
(72) Inventor: KASHIRIN, Alexandr Ivanovich, Kaluzhskaya obl., 249034 (RU); KLYUEV, Oleg Fedorovich, Obninsk, 249037 (RU); SHKODKIN, Alexandr Viktorovich, Kaluzhskaya obl., 249034 (RU)
(74) Representative: Jeck, Anton
(86) International application number: PCT/RU2006/000116
(87) International publication number: WO 2006/123965

(56) References cited:
- EP-A1- 0 189 709
- EP-A1- 0 261 973
- EP-A1- 1 369 498
- EP-A1- 1 445 033
- CA-C- 2 270 260
- DE-A1- 10 126 100
- DE-A1- 10 319 481
- RU-C1- 2 181 788
- RU-U1- 4 700
- US-A- 6 139 913
- US-B1- 6 402 050

## Description

### FIELD OF THE INVENTION

This invention relates to the technology of applying coatings to the surfaces, and in particular, to gas-dynamic methods of applying coatings with the use of an inorganic powder. It can be used in different branches of mechanical engineering, particularly for the restoration of the shape and dimension of metal parts, for the manufacturing and repair of metal parts to improve their impermeability or corrosion resistance or heat resistance or other property.

### BACKGROUND OF THE INVENTION

Gas-dynamic spray methods are the effective techniques for producing metal and mixed metal - ceramic coatings by the treating the substrate by a high - velocity jet of fine solid particles. In these methods the particles are accelerated in the high velocity gas stream by the drag effect. Only compressed gases, predominantly air, are used for particle acceleration without using any combustible.

Known in the art is a method and apparatus for applying coatings [U.S. Pat. No. 5,302,414 issued 1994]. With this method, a coating is applied by introducing metal powders into a compressed gas flow, accelerating the gas-powder mixture in a supersonic nozzle (a de Laval type nozzle) and directing the accelerated powder particles to the substrate. The accelerated particles impinge on the substrate while having kinetic energy sufficient for adhering to the substrate surface. The coatings are produced with powder particles having a particle size of from 1 to 50 microns. The powder particles neither melt nor begin to soften prior to impingement on the substrate and adhere to the substrate when their kinetic energy is transformed to a sufficient mechanical deformation.

The improvement of this method and apparatus [U.S. Pat. No. 6,139,913 issued 2000 and U.S. Pat. No. 6,283,386 issued 2001] includes the proper choice of the gas flow cross-section to allow for the formation of coatings by particles having a particle size up to 106 microns.

The main disadvantages of these methods are due to a powder is injected into the heated compressed gas flow prior to passage through the de Laval nozzle throat. Because the heated main gas flow (gas stream) is under high pressure, an injection of the powder requires expensive and complicated high pressure powder delivery (powder supply) systems. The powder particles and heated main gas both must pass through the throat of the nozzle, and the particles often stick to the walls of a diverging portion and a throat of the nozzle and clog the nozzle. This requires a complete shutdown of the system and cleaning of the nozzle. As a result, the gas temperature must be sufficiently low - such that no softening and sticking of the particles to the nozzle walls take place. That temperature often turns out to be insufficient for effective coating. Besides, when using the powders with hard particles, a considerable wear of the nozzle throat occurs, causing the early destroying of the nozzle.

The further prior art methods of coating [U.S. Pat. No. 6,756,073 issued 2004; RU 2205897, 2001; RU 2100474, 1997; U.S. Pat. No. 6,402,050 issued 2002] are free of these drawbacks. These inventions use a supersonic nozzle, and a preheated compressed gas is supplied to this nozzle. The gas, when passing through a converging portion, a throat and a diverging portion of the nozzle, accelerates and forms a supersonic flow in the nozzle. At the point following the nozzle throat (downstream of the throat), the powder particles are introduced into said flow. They are accelerated by the supersonic gas flow and directed to a surface of the base (substrate).

In these methods the powder particles do not pass through the nozzle throat. This allows the gas temperature to be increased with no fear that the particles will stick to the walls of the nozzle and clog or plug the nozzle throat. Since the velocity of the gas flow accelerating the powder particles is roughly proportional to the square root of the gas temperature, an increase of the gas temperature results in an increase of the velocity gained by the powder particles in the nozzle, and so, in an increase of the probability of their adherence to the substrate surface upon impingement. Thus, it has been possible to increase the efficiency of particle deposition.

But, due to the fact that the powder is introduced only downstream of the nozzle throat, the entire length of the nozzle portion available for the powder particle acceleration is considerably reduced. The reduced accelerating distance diminishes the growth of coating deposition efficiency which could be achieved owing to the increase in the gas temperature.

The most similar to the claimed solution is an apparatus and method reported in CA 2270260, 2004. The apparatus comprises a compressed gas heater; a supersonic nozzle (the de Laval nozzle) directly connected to the compressed gas heater and comprising a throat positioned between a converging portion and a diverging portion of the nozzle; a unit for supplying powders into the nozzle, the powder being introduced (injected) into the nozzle downstream of the nozzle throat.

In this apparatus, the powder particles do not pass through the nozzle throat, and hence, they do not wear its walls. This allows the use of the powders with hard ceramic particles. Moreover, since in the supersonic portion (positioned downstream of the throat), the gas temperature is significantly lower than in the subsonic portion (positioned in front of the throat) and in the nozzle throat, the apparatus allows to increase the compressed gas temperature without nozzle clogging by the particle sticking to the nozzle walls.

Nevertheless, due to the shift of the powder injection point downstream of the nozzle throat (i.e. powder introduction inside the nozzle rather than in front of it), the length of the nozzle portion available for particle acceleration is reduced. As a result, the final powder particle velocity reduces followed by the decrease of sprayed powder deposition efficiency.

Further information pertaining to the prior art can be found in EP 1 445 033 that discloses a kinetic spray tin coating process that enables the coating to withstand severe bending and stress without delamination. The method includes use of a low pressure kinetic spray supersonic nozzle having a throat located between a converging region and a diverging region. A main gas temperature is raised to from 1000 to 1300 degrees Fahrenheit and the coating particles are directly injected into the diverging region of the nozzle at a point after the throat. The particles are entrained in the flow of the gas and accelerated to a velocity sufficient to result in partial melting of the particles upon impact on a substrate positioned opposite the nozzle and adherence of the particles to the substrate. A nozzle is taught having a throat diameter of 1.5 to 3 mm, a diverging region with a length of 100 to 400 mm, and an exit end with a long dimension of 8 to 14 mm and a short dimension of 2 to 6 mm. It is taught to inject the particles into the diverging region at a distance of 12.7 mm to 127 mm from the throat.

### SUMMARY OF THE INVENTION

The object of present invention is an increase of sprayed powder deposition efficiency with the retention of the possibility to increase the compressed gas temperature and to use powders with hard particles.

The given object is accomplished by the fact that in the prior art apparatus for gas-dynamic applying coatings, comprising a compressed gas heater, a supersonic nozzle (the de Laval nozzle), directly connected to the gas heater and having a throat positioned between a converging portion and a diverging portion, a unit for supplying powders into the nozzle, wherein the powder injection components are placed down-stream of the nozzle throat, the unit for supplying powders into the nozzle has one or more powder feeders connected through conduits to the components for injection of one or more powders into the nozzle, and a nozzle portion positioned downstream of the powder injection components and intended for acceleration of the powders is made having parameters to suit the following relation: $0.015 < B \cdot \left(Sout/Sinj-1\right) / L < 0.03$
where
Sout - the area of the nozzle cross-section at the outlet;
Sinj - the area of the nozzle cross-section at the location of the powder injection components;
L - the length of the nozzle portion intended for acceleration of the powders;
B - the minimal dimension of the nozzle cross-section at the location of the powder injection components.

Depending on a shape and composition of the surface being treated and on the task to be accomplished upon coating, the nozzle can have a round or rectangular cross-section.

For the convenience during practical application of the apparatus, the nozzle portion intended for powder acceleration (acceleration portion) can be made as a replaceable element. In this case, it can be continuously divergent or have one or more cylindrical sections. The components for injection powders into the nozzle can be made as an orifice (orifices) in the nozzle wall or in the form of the tubes passing through the nozzle throat with the outlets being positioned downstream of (behind) the throat; with this, two or more components for injection powders can be made so as to ensure the powder supply equidistant from the nozzle throat.

To provide an easy change in the composition of a powder being sprayed, each feeder can be connected to its component for injection the powder into the nozzle. To simplify the construction, two or more feeders can be connected to the same component for injection the powder into the nozzle. For the convenience of apparatus practical use the compressed gas heating can be provided by electric heater.

The comparative analysis has shown that the claimed solution is distinguished from the prototype by the fact that a nozzle portion positioned downstream of the powder injection components and intended for acceleration of the powders has parameters to suit the following relation: $0.015 < B ⋅ \left(Sout/Sinj-1\right) / L < 0.03$
where
Sout - the area of the nozzle cross-section at the outlet;
Sinj - the area of the nozzle cross-section at the location of the powder injection components;
L - the length of the nozzle portion intended for acceleration of the powders;
B - the minimal dimension of the nozzle cross-section at the location of the powder injection components,
which makes it possible to judge the conformity of the invention to the criterion of novelty.

The given object can also be accomplished if in the prior art method of gas-dynamic applying coatings, comprising heating a compressed gas; supplying it into a supersonic nozzle (the de Laval nozzle) having a throat positioned between a converging portion and a diverging portion; forming a supersonic gas flow in the nozzle; injection a powder into the supersonic gas flow downstream of the nozzle throat (behind the throat); accelerating the powder by the gas flow in the nozzle; directing said accelerated powder to the substrate surface; and forming a coating, the powder is injected into the supersonic gas flow downstream of the throat, said powder comprising the particles of one or more substances, one of which being a metal and/or an alloy, the gas flow downstream of the nozzle throat being formed to suit the following relation: $0.015 < B ⋅ \left(Sout/Sinj-1\right) / L < 0.03 ,$
where
Sout - the area of the gas flow cross-section at the nozzle outlet;
Sinj - the area of the gas flow cross-section at the point of powder injection;
L - the length of the gas flow in the nozzle from the powder injection point to the nozzle outlet;
B - the minimal dimension of the gas flow cross-section at the point of powder injection.

Depending on the coating properties required, a metal powder, and/or a mechanical mixture of ceramic and metal powders is employed as a powder for forming the coating, or several powders of different hardness are injected into the supersonic flow at the same time, a ceramic powder being employed as one of the powders. The particle size of the powders used, both metal and ceramic ones, ranges from 1 to 100 micrometers.

The gist of the present invention resides in the following.

Upon gas-dynamic spraying of powder materials, a coating is formed by the separate particles, which upon impingement on the base are adhered to its surface basically due to the transformation of their kinetic energy to bonding energy.

Therefore, the possibility of the particle adherence to the surface depends mainly on their velocity. The higher is the velocity of each particular particle, the higher is the possibility of its adherence to the substrate surface, and hence, the higher is powder spraying efficiency (deposition efficiency) as a whole.

In all apparatuses for gas-dynamic applying coatings of powder materials the particles are accelerated in the high velocity gas flow by the drag effect. Accelerating Stokes force is proportional to the difference of the velocity of gas flow and that of the particles. For a limited acceleration time the particles never run up to the velocity of a gas flow and always lag behind it. The longer the particle is in the gas flow, the less is its lag, i.e. a velocity of the particle approaches that of gas.

It would seem obvious that one should elongate, as far as possible, a nozzle portion intended for acceleration of powder particles (an acceleration portion which is a nozzle portion extending from the point of powder injection up to the nozzle outlet). In that case, the particles move in the gas flow longer, and hence, they are accelerated to higher velocity.

In practice, it turned out to be not nearly so. A gradual increase in the length of the nozzle acceleration portion initially results in an increase in the particle velocity and greater efficiency of spraying the powder onto the substrate. However, on further increase in the length of the acceleration portion, the decrease of particle deposition efficiency is observed.

At first sight, this could be attributed to retardation of the gas flow due to the gas flow friction on the nozzle walls. In fact, in the apparatuses for gas-dynamic spraying, highly extended nozzles are commonly used whose length is dozens of times greater than the nozzle cross-sectional dimensions. In this case, retardation of gas in the nozzle can be sufficient, and under gas deceleration below the particle velocity, the particles start to be retarded instead of being accelerated.

However, in actual practice it has been found that with increasing the length of the nozzle acceleration portion, the decrease of the deposition efficiency begins well before sufficient deceleration of gas in the nozzle. That is, with some extension of the nozzle acceleration portion, the velocity of gas in the nozzle remains much above that of the particles. So with such extension of the nozzle acceleration portion the powder particles in the nozzle must acquire higher velocity. But in practice, the actual spraying efficiency unexpectedly decreases.

This effect can be explained by the following.

The powder particles injected into a gas flow necessarily have a velocity component directed across the flow. This velocity component arises both straight on introduction of the particles into the flow and in subsequent stages of particle trajectory evolution in the flow due to collision of the particles and their scattering by discontinuities of the flow. The acceleration of the particles in the nozzle is effected by a high-velocity gas flow directed along the nozzle axis. Therefore, practically straight after introduction of the powder particles into the accelerated gas flow, a transverse component of powders velocity becomes much less than the longitudinal one (directed along the gas flow). However, it exists and is assumed by the authors to be of considerable importance. The point is that the particles whose velocity is not directed strictly along the nozzle axis can impinge on the nozzle walls, and naturally, lose some of their longitudinal velocity. Besides, near the nozzle walls there is always a boundary gas layer the velocity of which is sufficiently lower than that of the main gas flow. The particles having a transverse velocity component can get into this boundary layer and slow down therein.

At the same statistical dispersion of transverse velocities of the particles, a probability that the particles get into a near-wall area of the nozzle increases with reducing the nozzle cross-section and increasing its length. As a consequence, the observed effect turned out to be connected not only with the nozzle length but with the cross section of its acceleration portion and with the degree of its divergence (increase of cross-sectional area of the nozzle in the direction of the gas flow).

Thus, with extending the nozzle acceleration portion, two processes take place at one time. Firstly, there is an increase in the velocity of the particles that have not impinged on the nozzle walls. Secondly, there is an increase in the number of the particles that have reached the near-wall area and partially lost the velocity upon the impingement on the nozzle walls or upon deceleration in the gas boundary layer.

As a result, with increasing the length of the nozzle, the maximal velocity of the particles in the nozzle increases, whereas the ratio of these high-velocity particles in the overall flow of the particles goes down. Consequently, as the nozzle is made longer, first, an average velocity of the particles increases and then it slows down.

In practice, this effect manifests itself through a variation in powder deposition efficiency. In the process, the powder deposition efficiency varies only slightly over a definite range of the nozzle acceleration portion length. In this range, the processes of the particle acceleration by the gas flow and deceleration in the near-wall area of the nozzle are approximately equalized, and so, there is only slight variation in the powder deposition efficiency.

Numerous experiments have shown that this effect of equalizing the particle acceleration and deceleration processes is achieved by the choice of a definite geometric parameters of the nozzle acceleration portion, and namely,

Numerous experiments have shown that this effect of equalizing the particle acceleration and deceleration processes is achieved if a definite relation between the basic geometric parameters of the nozzle acceleration portion is ensured, and namely, $0.015 < B ⋅ \left(Sout/Sinj-1\right) / L < 0.03 ,$
where.
Sout - the area of the gas flow cross-section at the nozzle outlet;
Sinj - the area of the gas flow cross-section at the point of powder injection;
L - the length of the gas flow in the nozzle from the powder injection point to the nozzle outlet;
B - the minimal dimension of the gas flow cross-section at the point of powder injection.

When the nozzle's parameters were beyond the bounds of the said limits, the decrease of the deposition efficiency was observed. In particular, with fixed values of the minimal cross-sectional dimension and cross-sectional area of the nozzle, excessively short and excessively long nozzles offered lower deposition efficiency than those whose length was kept within the said range.

The indicated features have not been revealed in other engineering solutions on studying the prior art. Thus, the claimed solution meets the inventive criterion and inventive step.

### BRIEF DESCRIPTION OF THE DRAWINGS

The invention is illustrated in the accompanying drawings, in which Fig.1 is a structural arrangement of the claimed apparatus and Fig.2 is a schematic illustration of the supersonic nozzle. The apparatus comprises a compressed gas heater 1, a nozzle 2 with a nozzle throat 3, a powder supply unit comprising powder feeders 4 and powder injection components 5 connected to the feeders by means of pipes 6, a nozzle acceleration portion 7 positioned downstream of the powder injection components up to the nozzle outlet and made, for instance, as a replaceable element 8 (Fig.2) also comprising a cylindrical section 9 (Fig.2).

In operation, a compressed gas is delivered to the heater 1 to be heated to the required temperature. The heated gas enters the supersonic nozzle 2, wherein it sequentially passes through a converging portion, the throat 3 and a diverging portion of the nozzle, and accelerates up to a supersonic velocity. The powders to be sprayed are introduced into this supersonic gas flow through the powder injection components 5. The powder particles are accelerated by a high-velocity gas flow at the nozzle acceleration portion 7 and then they are directed to the substrate surface.

Depending on a shape and composition of the surface being treated and on the task to be accomplished upon coating, the nozzle can have a round or rectangular cross-section.

For the use of the powders of hard substances (in particular, ceramic particles), the nozzle acceleration portion can be made, in full or in part, as a replaceable element 8 (Fig.2). In this case, the nozzle portion worn by the hard particles can be easily replaced.

To compensate for retardation of the gas flow against the nozzle walls, the nozzle acceleration portion can be made, in full or in part, divergent.

For simplification of the nozzle construction, its acceleration portion can have one or more cylindrical sections 9 (Fig.2).

Depending on the particular structure of the nozzle, one or more components for powder injection can be made as orifices (Fig.1) in the nozzle wall or as the tubes passing through the nozzle throat (Fig.2). Two or more powder injection components can be made so as to ensure the powder supply equidistant from the nozzle throat (Fig.1).

To provide an easy change of the powder being sprayed, each feeder can be connected to separate powder injection component. Two or more powder feeders can be connected to the same powder injection component to simplify the apparatus structure (Fig.1).

For the convenience of apparatus practical use the compressed gas heater can be electrical.

### SPECIFIC EXAMPLES OF THE INVENTION

The present invention is illustrated by the following specific examples given in Table 1 and Table2 below.

Table 1 presents the results of coating weights measurements. The coatings were sprayed with the round nozzles of different length at constant values of B=3.6 mm, Sinj = 10 mm² and Sout = 18 mm². The temperature of compressed air was 370°C. In all the cases, the same quantity of the powder was used, comprising:
a) aluminum (60%, wt.) and aluminum oxide (40%, wt.) particles,
b) copper (70%, wt.) and aluminum oxide (30%, wt.) particles,
c) zinc (60%, wt.) and aluminum oxide (40%, wt.) particles.

**Table 1**

| | L, mm | 190 | 170 | 150 | 130 | 110 | 90 |
|---|---|---|---|---|---|---|---|
| | B·(Sout/Si nj -1)/L | 0.015 | 0.017 | 0.019 | 0.022 | 0.026 | 0.03 |
| | Coating mass, g | 12 | 14 | 15 | 15 | 13 | 11 |
| | Coating mass, g | 16 | 18 | 19 | 19 | 17 | 14 |
| | Coating mass, g | 11 | 12 | 13 | 13 | 12 | 11 |

Table 2 presents other results of coating weights measurements. The coatings were sprayed with rectangular nozzles of different length with constant values of B = 3.6 mm, Sinj = 15 mm² and Sout = 30 mm². In all the cases, the same quantity of the powder was used, comprising the particles of aluminum (60%, wt.) and aluminum oxide (40%, wt.). The temperature of compressed gas was as follows: a) 370°C, b) 450°C, and c) 520°C.

**Table 2**

| | L, mm | 200 | 180 | 160 | 140 | 120 | 100 |
|---|---|---|---|---|---|---|---|
| | B· (Sout/Sinj -1)/L | 0.015 | 0.017 | 0.019 | 0.021 | 0.025 | 0.03 |
| | Coating mass, g | 7 | 8 | 10 | 10 | 9 | 8 |
| | Coating mass, g | 12 | 13 | 13 | 13 | 12 | 10 |
| | Coating mass, g | 16 | 17 | 18 | 18 | 15 | 12 |

In both cases compressed gas was an air under pressure of 7 bars.

Both tables demonstrate that as the dimensions relation approaches the limiting values, the coating mass diminishes, indicating the decrease of the powder deposition efficiency.

## Claims

1. An apparatus for gas-dynamic applying coatings comprising:
a compressed gas heater (1);
a supersonic nozzle (2) directly connected to the gas heater and having a throat (3) positioned between a converging portion and a diverging portion; and
a powder supply unit for supplying powders into the nozzle, the powder supply unit comprising powder injection components (5) placed downstream of the nozzle throat and one or more powder feeders (4) connected through conduits to the components for injection of one or more powders into the nozzle,
wherein
the nozzle has a nozzle acceleration portion (7) extending from the powder injection components to an outlet of the nozzle, the nozzle acceleration portion being intended for acceleration of the powders;
**characterized in that**
the nozzle acceleration portion has parameters to suit the following relation: $0.015 < B \cdot \left(Sout/Sinj-1\right) / L < 0.03$
where
Sout is the area of the nozzle cross-section at the outlet;
Sinj is the area of the nozzle cross-section at the location of the powder injection components;
L is the length of the nozzle acceleration portion;
B is the minimal dimension of the nozzle cross-section at the location of the powder injection components.

2. An apparatus according to claim 1 **characterized in that** the supersonic nozzle has a round cross-section.

3. An apparatus according to claim 1 **characterized in that** the supersonic nozzle has a rectangular cross-section.

4. An apparatus according to claim 1 **characterized in that** the nozzle acceleration portion is made in the form of a replaceable element (8).

5. An apparatus according to claim 1 **characterized in that** the nozzle acceleration portion is made divergent.

6. An apparatus according to claim 1 **characterized in that** the nozzle acceleration portion has one or more cylindrical sections (9).

7. An apparatus according to claim 1 **characterized in that** the powder injection components are made as orifices in the nozzle wall.

8. An apparatus according to claim 1 **characterized in that** one or more powder injection components are made in the form of the tube (6) passing through the nozzle throat with the outlets being positioned downstream of the throat.

9. An apparatus according to claim 1 **characterized in that** two or more powder injection components are made so as to ensure the powder injection equidistant from the nozzle throat.

10. An apparatus according to claim 1 **characterized in that** each powder feeder is connected to its component for injection of the powder into the nozzle.

11. An apparatus according to claim 1 **characterized in that** two or more powder feeders are connected to one component for injection of the powder into the nozzle.

12. An apparatus according to claim 1 **characterized in that** the gas heater is made electrical.

13. A method for gas-dynamic applying coatings using the apparatus of claim 1, comprising:
heating of a compressed gas;
supplying the heated gas into a supersonic nozzle (2) having a throat (3) positioned between a converging portion and a diverging portion;
forming a supersonic gas flow in the nozzle;
injecting a powder into the supersonic gas flow downstream of the nozzle throat;
accelerating the injected powder by the gas flow in the nozzle;
directing said accelerated powder to the substrate surface; and
forming a coating, wherein
the powder, having the particles of one or more substances, one of which being a metal and/or an alloy, is injected into the supersonic gas flow downstream of the throat.

14. A method according to claim 13 **characterized in that** a mechanical mixture of ceramic and metal powders is employed as the powder sprayed.

15. A method according to claim 13 **characterized in that** several powders having particles of different hardness are injected into the supersonic flow at the same time.

16. A method according to claim 13 **characterized in that** a ceramic powder is employed as one of the powders.

17. A method according to claim 14 **characterized in that** metal powders with the particle size from 1 to 100 microns are employed as the metal powder.

18. A method according to claim 16 **characterized in that** the powders of a particle size from 1 to 100 microns are employed as the ceramic powder.

## Patentansprüche

1. Vorrichtung zum gasdynamischen Aufbringen von Beschichtungen, wobei die Vorrichtung umfasst:
einen Druckgaserhitzer (1);
eine Überschalldüse (2), die direkt mit dem Gaserhitzer verbunden ist und die eine Verengung (3) aufweist, die zwischen einem konvergierenden Abschnitt und einem divergierenden Abschnitt positioniert ist; und
eine Pulverzuführungseinheit, um Pulver in die Düse zuzuführen, wobei die Pulverzuführungseinheit Komponenten (5) zur Pulvereinspritzung, die stromabwärts der Düsenverengung angeordnet sind, und ein oder mehrere Pulveraufgabevorrichtungen (4), die durch Leitungen mit den Komponenten zur Einspritzung von einem oder mehreren Pulvern in die Düse verbunden sind, umfasst,
wobei
die Düse einen Düsenbeschleunigungsabschnitt (7), der sich von den Komponenten zur Pulvereinspritzung bis zu einem Auslass der Düse erstreckt, aufweist, wobei der Düsenbeschleunigungsabschnitt dem Zweck der Beschleunigung der Pulver dient;
**dadurch gekennzeichnet, dass**
der Düsenbeschleunigungsabschnitt Parameter aufweist, um der folgenden Beziehung zu genügen: $0 , 015 < B * \left(Sout/Sinj-1\right) / L < 0 , 03$
wobei
Sout die Fläche des Düsenquerschnitts an dem Auslass ist;
Sinj die Fläche des Düsenquerschnitts an der Stelle der Komponenten zur Pulvereinspritzung ist;
L die Länge des Düsenbeschleunigungsabschnitts ist;
B die minimale Dimension des Düsenquerschnitts an der Stelle der Komponenten zur Pulvereinspritzung ist.

2. Vorrichtung nach Anspruch 1, **dadurch gekennzeichnet, dass** die Überschalldüse einen runden Querschnitt aufweist.

3. Vorrichtung nach Anspruch 1, **dadurch gekennzeichnet, dass** die Überschalldüse einen rechteckigen Querschnitt aufweist.

4. Vorrichtung nach Anspruch 1, **dadurch gekennzeichnet, dass** der Düsenbeschleunigungsabschnitt in der Form eines austauschbaren Elements (8) hergestellt ist.

5. Vorrichtung nach Anspruch 1, **dadurch gekennzeichnet, dass** der Düsenbeschleunigungsabschnitt divergent hergestellt ist.

6. Vorrichtung nach Anspruch 1, **dadurch gekennzeichnet, dass** der Düsenbeschleunigungsabschnitt einen oder mehrere zylindrische Abschnitte (9) aufweist.

7. Vorrichtung nach Anspruch 1, **dadurch gekennzeichnet, dass** die Komponenten zur Pulvereinspritzung als Öffnungen in der Düsenwand hergestellt sind.

8. Vorrichtung nach Anspruch 1, **dadurch gekennzeichnet, dass** eine oder mehrere Komponenten zur Pulvereinspritzung in der Form des Rohres (6) hergestellt sind, das durch die Düsenverengung verläuft, wobei die Auslässe stromabwärts der Verengung positioniert sind.

9. Vorrichtung nach Anspruch 1, **dadurch gekennzeichnet, dass** zwei oder mehrere Komponenten zur Pulvereinspritzung hergestellt sind, um zu gewährleisten, dass die Pulvereinspritzung von der Düsenverengung gleich weit entfernt ist.

10. Vorrichtung nach Anspruch 1, **dadurch gekennzeichnet, dass** jede Pulveraufgabevorrichtung mit ihrer jeweiligen Komponente zur Einspritzung des Pulvers in die Düse verbunden ist.

11. Vorrichtung nach Anspruch 1, **dadurch gekennzeichnet, dass** zwei oder mehr Pulveraufgabevorrichtungen mit einer Komponente zur Einspritzung des Pulvers in die Düse verbunden sind.

12. Vorrichtung nach Anspruch 1, **dadurch gekennzeichnet, dass** der Gaserhitzer elektrisch betrieben wird.

13. Verfahren zum gasdynamischen Aufbringen von Beschichtungen unter Verwendung der Vorrichtung nach Anspruch 1, das umfasst:
Erwärmen eines Druckgases;
Zuführen des erwärmten Gases in eine Überschalldüse (2), die eine Verengung (3) aufweist, die zwischen einem konvergierenden Abschnitt und einem divergierenden Abschnitt positioniert ist;
Bilden einer Überschallgasströmung in der Düse;
Einspritzen eines Pulvers in die Überschallgasströmung stromabwärts der Düsenverengung;
Beschleunigen des eingespritzten Pulvers durch die Gasströmung in der Düse;
Lenken des beschleunigten Pulvers auf die Substratoberfläche; und
Bilden einer Beschichtung, wobei
das Pulver, das die Partikel von einer oder von mehreren Substanzen aufweist, von denen eine ein Metall und/oder eine Legierung ist, in die Überschallgasströmung stromabwärts der Verengung eingespritzt wird.

14. Verfahren nach Anspruch 13, **dadurch gekennzeichnet, dass** eine mechanische Mischung aus keramischen Pulvern und Metallpulvern als das gesprühte Pulver eingesetzt wird.

15. Verfahren nach Anspruch 13, **dadurch gekennzeichnet, dass** mehrere Pulver mit Partikeln unterschiedlicher Härte gleichzeitig in die Überschallströmung eingespritzt werden.

16. Verfahren nach Anspruch 13, **dadurch gekennzeichnet, dass** ein keramisches Pulver als eines der Pulver eingesetzt wird.

17. Verfahren nach Anspruch 14, **dadurch gekennzeichnet, dass** Metallpulver mit der Partikelgröße von 1 bis 100 Mikrometer als das Metallpulver eingesetzt werden.

18. Verfahren nach Anspruch 16, **dadurch gekennzeichnet, dass** die Pulver einer Partikelgröße von 1 bis 100 Mikrometer als das keramische Pulver eingesetzt werden.

## Revendications

1. Appareil pour l'application gaz dynamique de revêtements, comprenant :
un dispositif de chauffage de gaz comprimé (1) ;
une buse supersonique (2) qui est directement connectée au dispositif de chauffage de gaz et présentant un col (3) positionné entre une partie convergente et une partie divergente ; et
une unité de fourniture de poudre pour introduire des poudres dans la buse, l'unité de fourniture de poudre comprenant des composants d'injection de poudre (5) placés en aval du col de la buse, et un ou plusieurs dispositif(s) d'alimentation de poudre (4) connecté(s) à travers des conduits aux composants pour l'injection d'une ou de plusieurs poudre(s) dans la buse,
dans lequel la buse comprend une partie d'accélération de buse (7) qui s'étend à partir des composants d'injection de poudre jusqu'à une sortie de la buse, la partie d'accélération de buse étant destinée à accélérer les poudres,
**caractérisé en ce que** la partie d'accélération de buse présente des paramètres pour respecter la relation suivante : $0 , 015 < B ⋅ \left({S}_{out}/{S}_{inj}-1\right) / L < 0 , 03$
dans laquelle :
Sₒᵤₜ est la surface de la section transversale de la buse à la sortie ;
Sᵢₙⱼ est la surface de la section transversale de la buse à l'endroit des composants d'injection de poudre ;
L est la longueur de la partie d'accélération de buse ; et
B est la dimension minimale de la section transversale de la buse à l'endroit des composants d'injection de poudre.

2. Appareil selon la revendication 1, **caractérisé en ce que** la buse supersonique présente une section transversale ronde.

3. Appareil selon la revendication 1, **caractérisé en ce que** la buse supersonique présente une section transversale rectangulaire.

4. Appareil selon la revendication 1, **caractérisé en ce que** la partie d'accélération de buse est conçue sous la forme d'un élément remplaçable (8).

5. Appareil selon la revendication 1, **caractérisé en ce que** la partie d'accélération de buse est divergente.

6. Appareil selon la revendication 1, **caractérisé en ce que** la partie d'accélération de buse présente une ou plusieurs section(s) cylindrique(s) (9).

7. Appareil selon la revendication 1, **caractérisé en ce que** les composants d'injection de poudre sont prévus comme des orifices dans la paroi de la buse.

8. Appareil selon la revendication 1, **caractérisé en ce qu'**un ou plusieurs composant(s) d'injection de poudre est (sont) prévu(s) sous la forme du tube (6) qui passe à travers le col de la buse avec les sorties qui sont positionnées en aval du col.

9. Appareil selon la revendication 1, **caractérisé en ce que** deux ou plus de deux composants d'injection de poudre sont conçus de manière à assurer une injection de poudre équidistante à partir du col de la buse.

10. Appareil selon la revendication 1, **caractérisé en ce que** chaque dispositif d'alimentation de poudre est connecté à son composant pour l'injection de la poudre dans la buse.

11. Appareil selon la revendication 1, **caractérisé en ce que** deux ou plus de deux dispositifs d'alimentation de poudre sont connectés à un composant pour l'injection de la poudre dans la buse.

12. Appareil selon la revendication 1, **caractérisé en ce que** le dispositif de chauffage de gaz est de nature électrique.

13. Procédé pour l'application gaz dynamique de revêtements en utilisant l'appareil selon la revendication 1, comprenant les étapes suivantes :
chauffer un gaz comprimé ;
introduire le gaz chauffé dans une buse supersonique (2) comprenant un col (3) qui est positionné entre une partie convergente et une partie divergente ;
former un écoulement de gaz supersonique dans la buse ;
injecter une poudre dans l'écoulement de gaz supersonique en aval du col de la buse ;
accélérer la poudre injectée par l'écoulement de gaz dans la buse ;
diriger ladite poudre accélérée vers la surface du substrat ; et
former un revêtement,
dans lequel la poudre, qui contient des particules d'une ou de plusieurs substance(s), dont l'une est un métal et/ou un alliage, est injectée dans l'écoulement de gaz supersonique en aval du col en utilisant l'appareil selon la revendication 1.

14. Procédé selon la revendication 13, **caractérisé en ce qu'**un mélange mécanique de poudres de céramique et de métal est employé pour la poudre pulvérisée.

15. Procédé selon la revendication 13, **caractérisé en ce que** plusieurs poudres présentant des particules de dureté différente sont injectées dans l'écoulement supersonique en même temps.

16. Procédé selon la revendication 13, **caractérisé en ce qu'**une poudre de céramique est employée pour l'une des poudres.

17. Procédé selon la revendication 14, **caractérisé en ce que** des poudres de métal présentant une taille de particule de 1 micron à 100 microns sont employées pour la poudre de métal.

18. Procédé selon la revendication 16, **caractérisé en ce que** des poudres présentant une taille de particule de 1 micron à 100 microns sont employées pour la poudre de céramique.
